

# UNITED STATES PATENT OFFICE.

ALBERT G. MANNS, OF OCONOMOWOC, WISCONSIN, ASSIGNOR TO ALBERT O. TROSTEL,  
OF MILWAUKEE, WISCONSIN.

## PROCESS FOR DETANNING.

967,215.

Specification of Letters Patent. Patented Aug. 16, 1910.

No Drawing.

Application filed April 5, 1909. Serial No. 488,005.

To all whom it may concern:

Be it known that I, ALBERT G. MANNS, a citizen of the United States, residing at Oconomowoc, in the county of Waukesha 5 and State of Wisconsin, have invented a certain new and useful Process for Detanning, of which the following is a specification.

This invention relates to a process for detanning leather, and refers more specifically to a process for detanning chrome 10 tanned leather or leather waste, etc.

The salient object of the invention is to provide a process whereby chrome tanned leather or leather waste may be thoroughly 15 detanned without impairing, or substantially impairing, its strength or structure, so that upon the completion of this detanning process it will be restored practically to its original untanned condition and the product 20 may thereafter be utilized for any of the numerous uses to which untanned hides or scraps of hides might be converted.

Other objects of the invention are to provide a process which is simple, economical, 25 and by means of which the chemical used in tanning the leather may be recovered as a by-product; to provide a process which is admirably suited for placing the material treated in condition for making either good 30 gelatin or high grade glue; to provide a process which is especially applicable for treating finely comminuted waste leather without loss or waste of the material; to provide a process which may be carried 35 through in a comparatively short time, and in general to provide an improved process of the character referred to.

In the manufacture and working up of chrome tanned leather there is a comparatively large percentage of so-called waste, 40 which has heretofore been of little or no value because of the lack of any suitable process for utilizing such waste. Such waste includes so-called skivings, splits, 45 trimmings, skifings, shavings, thick pieces torn off in shaving or other working of skins, and inferior and rejected pieces of leather. Moreover, in making chrome tanned leather for grain finish there usually 50 results a certain proportion of hides which turn out to be unsatisfactory for this kind of leather,—the defective character of the 55 hides being only determinable by tanning them, and these hides can be advantageously detanned by my process and then retanned

by some other process, as for example to produce a flesh finished leather. Where the waste is in the form of scraps or shavings, unsuitable for use as leather, the detanned product secured by my process may be converted into gelatin, glue or even into animal food, since the product is, as above stated, returned substantially to its original animal condition.

The preferred way of carrying out my process is as follows: I first subject leather or leather waste to a bath or treatment of hot water, which rapidly softens the material and puts it in condition for the subsequent chemical treatment to affect it rapidly and uniformly. The hot water treatment is continued until the material is all thoroughly penetrated and softened. I next treat the material in a bath of a weak alkaline solution, which has the effect of loosening the chrome so that it will readily and thoroughly dissolve in the subsequent acid treatment. For this chemical bath I prefer to use lime water,—not milk of lime, because the use of the latter results in mixing the mineral lime into the finely comminuted and powdered waste to such an extent that a substantial percentage of it is inevitably lost in the subsequent washing out of the lime, besides making it more difficult to separate the alkali and lime from the material being treated. Ordinarily the lime water treatment will cover a period of from six to twelve hours. I next remove the lime water and preferably also wash the material with the water so as to minimize the amount of alkali remaining in the material to be neutralized. I next subject the material to an acid treatment, which dissolves the chrome and extracts it from the animal fiber. For this purpose I use a weak solution,—say a one to two per cent. solution, of sulfuric or sulfurous acids. Preferably, where a light colored product is desired, I use sulfurous acid solution, or a mixture of sulfurous and sulfuric acids, because this, to some extent, bleaches at the same time that it dissolves out the chrome. After the acid has thoroughly dissolved the chrome, this bath is drained off, and inasmuch as it will contain practically all of the chrome, the latter may be recovered from the drawn off liquid by any suitable process known to chemists. The material is now again washed to remove excess of acid,

60

70

75

80

85

90

95

100

105

110

and then the remaining acid neutralized by a second treatment with weak alkaline solution, preferably lime water, after which the material is washed and the detanning process thus completed. To make glue or gelatin, the detanned material will be afterward boiled in the usual manner, while if it is to be retanned it may be retanned by an ordinary tanning process.

10 The detanning process above described results in completely (or at least to all practical intents) freeing the leather from the tanning chemicals, and this without, so far as I have been able to determine, in any 15 wise impairing the tissue structure, strength or original character of the hide material. Pieces of leather detanned by the above process, and then retanned, appear to take the second tanning as perfectly and in precisely the same manner as though being tanned for the first time.

In the case of detanning freshly tanned hides, for the purpose of retanning by a different process, for example, the preparatory step of soaking up the leather may, of course, be omitted, since the leather will not be in dry and hard condition.

While I have hereinbefore indicated the preferred chemicals, and indicated these in 30 the proportions which I find best suited to secure the desired results, nevertheless different equivalent chemicals can be substituted, and the proportions varied within reasonable limits, without departing from 35 the spirit of the invention.

An important characteristic of the present invention is that throughout the entire series of steps the leather is at no time treated drastically with chemical, nor is any step of 40 the treatment continued so long as to result in impairing the tissue structure of the material.

I claim as my invention:

1. The improved process of detanning and 45 restoring mineral tanned leather to its original untanned condition, which consists in subjecting the leather material to treatment in a weak alkaline solution substantially free from undissolved mineral matters until 50 the leather is thoroughly impregnated throughout, next substantially separating the alkaline solution from the leather and subjecting the latter to a treatment with an acid having an effective strength, over 55 and above that necessary to neutralize the alkali remaining in the batch, of not much less than 1% and so weak as to be incapable

substantially attacking the animal matter during the period that it requires to completely dissolve the mineral tanning material, and continuing this step of the treatment until the tanning chemical has been thoroughly dissolved, then, before the animal matter has been appreciably attacked by the chemical, substantially removing the 65 last mentioned solution.

2. The improved process of detanning and restoring mineral tanned leather to its original untanned condition, which consists in subjecting the leather material to treatment 70 in a weak alkaline solution substantially free from undissolved mineral matters until the leather is thoroughly impregnated therewith throughout, next substantially separating the alkaline solution from the leather 75 and subjecting the latter to a treatment with an acid having an effective strength, over and above that necessary to neutralize the alkali remaining in the batch, of not much less than 1% and so weak as to be incapable 80 of substantially attacking the animal matter during the period that it requires to completely dissolve the mineral tanning material, continuing this step of the treatment until the tanning chemical has been thoroughly dissolved, then, before the animal 85 matter has been appreciably attacked by the chemical, substantially removing the last mentioned solution, and subjecting the material to a neutralizing treatment with a second weak alkaline solution until it remains alkaline, and finally washing out the free chemicals.

3. The process of detanning chrome or analogous mineral tanned leather or leather 95 waste, which consists in first subjecting the material to a hydrous bath until thoroughly soaked throughout, next subjecting the material to a treatment in a bath of lime water substantially free from suspended lime, next 100 separating the material from the lime water and subjecting it to a treatment in an acid solution of a strength not greater than 10% and not less than 1%, next removing the free acid solution and subjecting the material to 105 treatment with a neutralizing weak alkaline solution and thereby rendering the batch alkaline, and finally washing out the free chemicals.

ALBERT G. MANNS.

Witnesses:

ALBERT H. GRAVES,  
EMILIE ROSE.